# EUROPEAN PATENT APPLICATION

(11) **EP 4 261 343 A1**
(43) Date of publication of application: **18.10.2023**
(21) Application number: 22168234.7
(22) Date of filing: 13.04.2022
(51) Int. Cl.: D21C 3/02

(54) **CONVERSION OF BIOMASS RESIDUES INTO BIO-OIL**

(71) Applicant: SCA Forest Products AB, 85188 Sundsvall (SE)
(72) Inventor: KUGGE, Christian, 85231 Sundsvall (SE); EDLING HULTGREN, Anders, 85644 Sundsvall (SE); KOLAR, Milan, 85468 Sundsvall (SE)
(74) Representative: Weickmann & Weickmann PartmbB

(57) **Abstract**

The present invention relates to the production of a lignin-containing process stream by subjecting a biomass residue to a treatment under strong alkaline conditions and obtaining a lignin-containing process stream from the reactor.

## Description

The present invention relates to the production of a lignin-containing process stream by subjecting biomass residues to a treatment under strong alkaline conditions and obtaining a lignin-containing process stream from the reactor.

Lignin is one of the two major components of lignocellulose in plants. Structurally it is a class of complex cross-linked phenolic polymers. From an energy point of view, lignin has a high C/O ratio and accounts for a substantial proportion of carbon-based energy in lignocellulose. In the past however, lignin has only been considered as byproduct of the pulp and paper industry. Only a minor amount of lignin produced by the pulp and paper industry was utilized commercially and the remainder was used as a low-value fuel. Recently, efforts have been made to recover lignin and convert it to bio-oil.

Lignin may be recovered from hardwood, softwood but also from young plants, annual plants or energy crops. For bio-oil production, lignin from softwood, such as pine or spruce, or hardwood, such as birch, is used so far. Softwoods have a higher content of lignin than hardwoods.

WO 2004/106624 A1 discloses the production of pulp and lignin from a lignocellulosic material, comprising the impregnation of a lignocellulosic material with acid and acidic depolymerization of lignin before alkaline treatment. The alkaline digestion step is performed under mild conditions, i.e., at a temperature of less than 100°C.

WO 2020/084196 A1 discloses a process for extracting valuable components from a tannin-rich bark raw-material by carrying out an alkaline cooking step, followed by acid precipitation to separate valuable components from the remaining bark pulp. Alkaline cooking is carried out at relatively mild alkali conditions, i.e., 14-20% effective alkali charge. Depolymerization of lignin is not disclosed.

WO 2020/245071 A1 discloses the production of pulp for tissue products. The starting material is eucalyptus bark chips which have been pre-extracted with an ethanol-water mixture. The extracted bark chips are subjected to an alkali treatment at effective alkali charge of 22%. The digestion time is 200 minutes or longer and the temperature from 17-170°C. Depolymerization of lignin is not disclosed.

An object of the present invention was to provide economically feasible methods for the production of lignin and a bio-oil comprising depolymerized lignin.

### Summary of the invention

The present invention provides a novel process for producing a lignin-containing process stream by subjecting a biomass residue to a treatment under strong alkaline conditions and obtaining a lignin-containing process stream from the reactor.

The lignocellulosic biomass residue used in accordance with the present invention is generally referred to as low value lignocellulosic biomass.

The process may combine the use of lignocellulosic biomass residues with the depolymerization of lignin and optional production of biofuel from the depolymerized lignin.

A first aspect of the invention relates to a method for producing a lignin-containing process stream, comprising the steps of:
(a) providing a lignocellulosic biomass residue;
(b) introducing the biomass into a reactor;
(c) subjecting the biomass in the reactor to a treatment in the presence of an alkali source at elevated temperature, wherein the effective alkali charge is at least about 25%, wherein the temperature is at least about 150°C, and wherein the treatment time is at least about 1 h;
(d) obtaining a lignin-containing process stream from the reactor; and
(e) optionally removing char from the lignin-containing process stream.

The lignocellulosic biomass residue may, e.g., be sawdust, bark, branches, needles, young plants and/or straw. In certain embodiments, the lignocellulosic biomass residue is selected from sawdust, wood flour, wood chips, bark, branches, leaves, needles, or any mixture thereof.

In certain embodiments, the lignin-containing process stream obtained in step (d) or (e) is a black liquor, particularly a black liquor that does not comprise substantial amounts of solid pulp.

In certain embodiments, the lignin-containing process stream obtained in step (d) comprises solid pulp, particularly low-grade solid pulp, particularly wherein the pulp yield is from about 20% to about 45% based on dry feed of lignocellulosic biomass residue, and/or wherein the low-grade solid pulp has a Kappa number of about 50 or less, particularly of about 30 or less, more particularly of about 5 to about 20.

In a further aspect, the invention relates to a method that ultimately allows to obtain a bio-oil composition from the lignin-containing process stream obtained in step (d) described above. In certain embodiments, the lignin-containing process stream is subjected to a lignin-depolymerization step whereby a bio-oil containing process stream is obtained. From the bio-oil containing process stream a bio-oil composition may be obtained wherein the bio-oil composition comprises depolymerized lignin. The bio-oil composition may be subjected to further treatment steps including distillation and/or hydrotreatment.

In yet a further aspect, the invention relates to a bio-oil composition obtained by a method or process as described herein.

### Detailed Description

The present invention provides a novel process for the production of a lignin-containing process stream from lignocellulosic biomass residue by subjecting it to a treatment in the presence of an alkali source at elevated temperature.

In a first step (step (a)) of the new process, a lignocellulosic biomass residue, such as sawdust, wood flour, bark, branches or needles from softwood and/or hardwood or any mixture thereof is provided. In a subsequent step (step (b)), the biomass is fed to a reactor, e.g., batch-wise or continuously. Once in the reactor, the biomass is, according to step (c) of the new process, cooked in the presence of an alkaline solution, for example, white liquor, NaOH or KOH to produce a high yield lignin-containing process stream.

In a further process step (step (d)), the lignin-containing process stream is obtained from the reactor.

Optionally, a further step (e) may be performed, by which char is removed from the lignin-containing process stream obtained after step (d).

Depending on the treatment conditions, the lignocellulosic biomass residue can be completely liquefied in the reactor or converted to a process stream containing pulp. The basics of these two approaches are described below.

Both approaches differ from a conventional cooking process for production of pulp. In the process of the invention, the conditions (particularly temperature and alkaline levels) are very harsh, and the focus is to recover lignin, cellulose and hemicellulose in the process stream. In contrast to a conventional pulp manufacturing process, where the target is to produce pulp with high yield and high strength, the recovery of pulp is not crucial in the process of the invention. If a pulp fraction is produced, it is typically a fraction suitable for, for example, ethanol production. Such a pulp is sometimes referred to as being a low value fraction, as compared to a pulp produced by a conventional pulp manufacturing process.

The process stream obtained after step (d) or (e) of the new process is especially suitable for further treatment, e.g., in a depolymerization process for the production of a bio-oil. Due to the harsh conditions in the reactor utilized in the new process, the resulting process stream, e.g., a black liquor, will have higher content of lignin and extracted organic substances including converted cellulose and hemicellulose to cellulose- and hemicellulose-based derivatives (such as sugars and organic acids) when compared to a black liquor from a conventional pulping process. The higher content of lignin and cellulose- and hemicellulose-based derivatives results in a higher bio-oil yield after depolymerization of lignin. Further, the increased content of cellulose- and hemicellulose-based derivatives in the black liquor has a beneficial effect on the processability of the black liquor during and/or after lignin depolymerization.

The novel process of the present invention utilizes lignocellulosic biomass residue material. "Lignocellulosic biomass residue" as used herein relates to biomass of plant origin, e.g., from trees, bushes, weeds or grass or straw which is without or only low value for typical applications of plant-derived biomass such as manufacture of pulp and/or formed wooden parts such as furniture, panels, roofing, flooring, joinery etc.

The plant-derived lignocellulosic biomass residue may comprise wood residues and/or agricultural residues. In certain embodiments, agricultural residues such as straw (e.g. wheat, rye, barley, oat or rice straw), bagasse, cotton stalk and bran (e.g. wheat, rye, barley, oat or rice bran) may be utilized. In certain embodiments, the lignocellulosic biomass residue may be a tree-derived material, e.g., wood residue material such as sawdust, wood flour, or wood chips, bark, branches, leaves, needles, or any mixture thereof. The lignocellulosic biomass residue may be derived from softwood such as fir, pine, spruce, larch, hemlock, cedar and/or yew and/or from hardwood such as oak, beech, birch, eucalyptus etc.

In certain embodiments, the lignocellulosic biomass residue is wood residue material such as sawdust, wood flour and wood chips without a substantial amount, e.g., 10% (w/w) or more of bark material.

In certain embodiments, the lignocellulosic biomass residue is a softwood residue material comprising sawdust, wood flour, bark, branches, needles, or any mixture thereof.

In certain embodiments, the lignocellulosic biomass residue is softwood residue material, in particular softwood residue material comprising sawdust. In certain preferred embodiments, the lignocellulosic biomass residue essentially consists of softwood sawdust. In this context, "essentially consists of" means that at least about 95% (w/w), particularly about 97% (w/w), about 98% (w/w), about 99% (w/w), or even about 99.5% the lignocellulosic biomass residue is softwood sawdust. The remaining percentage to 100% (w/w) may consist of usual contaminations in sawdust known to the skilled person (such as ash and traces of bark).

In certain embodiments, the total biomass introduced into the reactor comprises at least about 50% (w/w), at least about 70% (w/w), or at least about 90% (w/w) of lignocellulosic biomass residue. In certain embodiments, the total biomass introduced into the reactor consists of lignocellulosic biomass residue.

In certain embodiments, the lignocellulosic biomass residue is introduced into the reactor without a pretreatment, e.g., a pretreatment selected from acid impregnation and/or extraction using an organic solvent, e.g., an ethanol/water mixture.

The reactor can be any suitable reactor capable of withstanding harsh alkaline conditions and high temperature.

In certain embodiments, a ratio of dry feed to liquid (w/w) from about 1:3 to about 1:10, particularly from about 1:4 to about 1:6, e.g., of about 1:5 is adjusted in the reactor. The term "liquid" refers to the liquid components present in the reactor forming a reactor medium. The liquid components comprise water, an alkali source and further optional components such as alcohols. The alkali source typically comprises a hydroxide, for example, Ba(OH)₂, NaOH and/or KOH. In certain embodiments, the alkali source may comprise a mixture of a hydroxide and a sulfide salt. In such a case, the alkali source may be white liquor, i.e., a mixture of NaOH and Na₂S.

The effective alkali charge in the reactor is adjusted to be at least about 25% on dry wood in order to provide sufficiently harsh alkaline conditions for digesting the lignocellulosic biomass residue. In certain embodiments, the effective alkali charge in the reactor is adjusted to least about 30%, particularly from about 35% to about 60% on dry wood. The effective alkali charge refers to the combined concentrations of NaOH and Na₂S (when present) as [NaOH] + ½ [Na₂S] (g/l) and later converted to % charge as mass alkali divided by mass dry wood.

The treatment conditions can be adapted to the desired degree of liquefaction of the lignocellulosic biomass residue. The temperature in the reactor is typically about 150°C or higher, e.g., about 150°C to about 280°C. In some embodiments, the temperature may be between about 150°C to about 200°C. In other embodiments, the temperature may be between about 170°C to about 230°C. In yet further embodiments, the temperature may be between about 200°C and about 250°C. In exemplary embodiments, the temperature may range between 175°C and 180°C, or between 200°C and 230°C. Pressures used are typically no lower than the saturation pressure of water at chosen operation temperature. Pressures further are typically such that no water is evaporated.

The treatment time is at least about 1 h, typically about 1 h to about 10 h, e.g. 1, 2, 3, 4, 5, 6, 7, 8, 9 or 10 h. In exemplary embodiments, the treatment time may be about 1 h, about 5 h or about 6 h.

In further exemplary embodiments, treatment may be performed for about 2 h at about 230°C, for about 5 h at about 155°C, for about 1.5 h at about 180°C, for about 5 h at about 200°C, for about 6 h at about 180°C, or for about 8 h at about 180°C, such as 178°C.

In this respect, the treatment conditions may also be defined by the Kraft H factor (also simply referred to as "H factor" in the following) that combines cooking temperature and time into a single variable that indicates the extent of reaction (cf. Pratima Bajpai, in Biermann's Handbook of Pulp and Paper, Third Ed., 2018, chapter 13.6) the content of which is herein incorporated by reference.

The H factor combines process temperature and residence time as the integral of the reaction rate with respect to time gives the H factor as shown below. $H = {\int }_{0}^{t} {e}^{\left(43.2-\frac{16115}{T}\right)} dt$

With the H factor one can control the severity of the pulping process and can compare it to a kraft pulp mill, which typically operates at a much lower H factor of 1000-1400 as well as a lower alkali charge of typically 20% on dry wood.

According to the present invention, the H factor particularly is at least about 2000. In certain embodiments, the H factor is at least about 4000, at least about 6000 or at least about 7000. In preferred embodiments, the H factor is at least about 8000. The maximum of the H factor according to the present invention is typically 5 000 000, particularly 3 000 000. In preferred embodiments, the H factor is about 1 000 000 or below.

As already mentioned above, according to a first approach of the invention the treatment conditions are adapted such that a substantially complete liquefaction of the lignocellulosic biomass residue is achieved. A resulting stream thus does not comprise a substantial amount of solid pulp. According to this approach, the H factor is at least about 2000 and at most about 3 000 000, particularly at most about 1 000 000, at most about 500 000, or at most about 200 000. In preferred embodiments according to this aspect, the H factor is in the range of about 8000 to about 1 000 000, particularly about 9000 to about 750 000, more particularly about 10000 to about 500 000.

According to a second approach of the invention, the treatment conditions are adapted such that a pulp, particularly a low-grade solid pulp, is obtained after the treatment. According to this approach, the H factor is in the range of about 2000 to about 13000. In preferred embodiments, the H factor is in the range of about 8000 to about 12000.

In the first approach as described above, the lignocellulosic biomass residue is subjected to treatment conditions resulting in a substantially complete liquefaction of the biomass within the reactor except in some cases for the formation of char, e.g., in a yield of about 15% or less or 10% or less based on the total amount of biomass introduced into the reactor, which can be removed from the process stream, e.g., by filtration. In certain embodiments, the lignin-containing process stream obtained in step (d) is a black liquor. In certain embodiments, the lignin-containing process stream obtained in step (d) does not comprise substantial amounts, e.g., about 5% (w/w) or less or about 1% (w/w) or less of solid pulp. In certain embodiments, the lignin-containing process stream obtained in step (d) contains about 0.1% (w/w) or less of solid pulp.

Benefits with this approach of utilizing a liquefied biomass are good processability, e.g., easy pumping, no removal of pulp and a high yield of bio-oil.

In certain embodiments, the treatment conditions for this approach are a temperature of about 180°C or higher, particularly from about 200°C to 280°C, and more particularly from about 210°C to about 240°C, and/or a treatment time from about 1 h to about 10 h. With a cooking time of 6 h, for example, cooking at 210°C equals an H factor of 114 000, and cooking at 240°C equals an H factor of 800 000. In specific embodiments, the reactor is a stirred reactor loaded with dry sawdust powder (wood flour) using Kraft mill white liquor as an alkali source, the temperature is at least 180 °C, the liquid/dry mass ratio is about 5/1 and/or the residence time is about 5 h or more. Diluted white liquor, e.g., 1/1 with water or black liquor also works to liquefy the biomass, e.g., sawdust. After the treatment in the reactor, the liquid may be cooled down and filtered to remove char. In certain embodiments, when a temperature of about 280 °C is used, the cooking time is about 1 h.

In certain embodiments, using the first approach, the lignocellulosic biomass residue is softwood residue material comprising sawdust and/or bark from softwood.

In the second approach, the treatment of biomass results in a process stream, e.g., a black liquor stream, comprising solid pulp. This can be done differently to a traditional Kraft pulp process as the novel process need not consider the strength of the resulting pulp. In certain embodiments, the pulp contains a low amount of lignin. The pulp can be released from the reactor under conditions where fibers are torn apart providing a low pulp strength, e.g., by creating a "steam explosion" when exiting the reactor. The low pulp strength is advantageous for certain applications, e.g., production of ethanol, while not being wanted in traditional Kraft pulping. Production of ethanol with a pure (low lignin content about 2% or less) low-strength pulp as starting material will be beneficial compared with a lignocellulosic starting material. Thereby, an acid hydrolysis of biomass and the difficult handling of hydrolysis lignin can be avoided.

In certain embodiments, the treatment conditions for this approach are a temperature between about 180°C and about 200°C, particularly between about 165°C to about 190°C, and more particularly between about 175°C to about 180°C, and/or a treatment time from about 3 h to about 8 h.

In certain embodiments of the second approach, the lignin-containing process stream obtained in step (d) or (e) comprises low-grade pulp with the tensile index of 60 kNm/kg. In certain embodiments, the pulp yield is from about 20% to about 45% based on dry feed of lignocellulosic biomass residue. In certain embodiments, the low-grade pulp has a Kappa number of about 50 or less, particularly of about 30 or less, more particularly of about 5 to about 20.

As already outlined above, the pulp may be separated from the lignin-containing process stream and optionally subjected to further processing, e.g., processing to sugar, biofuel such as ethanol, and/or biochemicals such as furan dicarboxylic acid (FDCA).

In certain embodiments of the second approach, the lignin-containing process stream obtained in step (d) or (e) is typically a black liquor. Compared to conventional black liquor, it comprises an increased content of dissolved organic matter, as can be determined, e.g., by comparison of the lignin content in pulp obtained from a kraft mill vs. pulp obtained according to the process of the present invention. Typically, the content of dissolved organic matter in the process stream of the invention is from about 60% to about 90% of dry solids content, particularly from about 65% to about 90% of dry solids content. In certain embodiments, the lignin-containing process stream obtained in step (d) or (e) comprises about 30 weight-% to about 50 weight-% of lignin, preferably >33 weight-%, more preferably >40 weight-% lignin based on the dry solid content within the process stream.

According to particular embodiments of the present invention, the lignin-containing process stream obtained after step (d) or (e) is subjected to a lignin depolymerization step in a depolymerization reactor whereby a bio-oil containing process stream is obtained. The bio-oil containing process stream may be subjected to further work-up and/or purification steps to obtain a bio-oil composition comprising depolymerized lignin. In order to obtain a bio-oil composition from the bio-oil containing process stream, one or more of the following steps may be performed:
(i) acidifying the bio-oil containing process stream;
(ii) adding crude tall oil;
(iii) adding a solvent and anti-solvent;
(iv) removing an aqueous phase, solvent and/or salts from the bio-oil containing process stream.

Where the bio-oil containing process stream is acidified, the acidification may, in exemplary embodiments, be carried out at a pH of from about 2 to about 5.

In certain embodiments, the lignin-containing process stream obtained in step (d) or (e) is subjected to a lignin-depolymerization step without addition of further components. In certain embodiments, the lignin-containing process stream obtained in step (d) or (e) is subjected to a lignin-depolymerization step with addition of further components, e.g., a conventional Kraft black liquor, lignin derived components and/or non-lignin derived components. Lignin derived components may include solid lignin powder and/or a depolymerized and partially hydrotreated, e.g., a partly deoxygenated and partly desulfurized bio-oil. Non-lignin derived components may include a fatty acid, particularly a rosin containing oil and more particularly tall oil and any product derived therefrom comprising rosin constituents, particularly resin acids, e.g., abietic acid and/or pimaric acid. For example, the rosin containing oil may be selected from crude tall oil and fractions of crude tall oil such as tall oil pitch, tall oil rosin, tall oil fatty acids, crude sulphate turpentine and/or any combination thereof.

The lignin depolymerization reaction is carried out in a reactor under conditions of elevated temperature and elevated pressure, which are suitable for conducting the depolymerization reaction.

The depolymerization reactor may be kept at a temperature between about 150°C and about 350°C, particularly between about 210°C and about 290°C, more particularly between about 230° and 250°C and/or at a pressure between about 5 bar and about 180 bar, particularly between about 15 bar and about 120 bar, optionally in the presence of a gas such as H₂, CO or H₂ or H₂/CO, particularly in the presence of H₂, and optionally in the presence of a catalyst.

The depolymerization reactor may be the same reactor as the reactor of the alkali treatment or, alternatively, the depolymerization reactor may be a separate reactor.

For the depolymerization of lignin a wide range of catalysts can be used such as a noble metal on a support such as a carbon-based support, e.g., activated carbon, charcoal, graphene, carbon nanotubes, or graphite, or a metal oxide-based support such as alumina, aluminum phosphate, zeolite, hydrotalcite, hydroxyapatite, magnesium oxide, zirconia, titanium dioxide, ceria, chromite, or molybdite. Other possible catalysts are transition metals such as V, Cr, Fe, Co, Ni, Cu, Zn, Zr, Nb, Mo and W or transition metal oxides such as NiO on any of the previously mentioned supports, as well as unsupported metal, metal oxide, metal carbide or metal nitride particles wherein the metal is particularly a transition metal such as Ni or Mo, which may be doped with another transition metal. Further unsupported catalysts that are suitable include Co-Mo-S, MoS₂, VS₂, Ni-Mo and Fe-Cu catalysts.

Suitable lignin depolymerization procedures are described in co-owned patent applications WO 2017/048163 A1, WO 2017/048164 A1, WO 2020/161313 A1, WO 2020/161323 A1, WO 2022/002774 A1 and WO 2022/002775 A1, the contents of which are herein incorporated by reference.

After lignin depolymerization, the bio-oil containing process stream may subjected to one or more additional treatment steps, e.g., work-up and/or purification steps, for example, acidifying the bio-oil containing process stream, e.g., with an acidifying agent selected from H₂SO₄, CO₂, SO₂, acidic process water having a pH of about 1 to about 3 or any combination thereof; adding a rosin containing oil such as crude tall oil to the bio-oil containing process stream; adding a solvent suitable to at least partially dissolve lignin components, such as ethanol or methanol, to the process stream; and/or removing an aqueous phase, solvent and/or salts from the bio-oilcontaining process stream.

According to particular embodiments of the present invention, the added solvent has two functions, being a solvent for the lignin and an anti-solvent for the salts. In particular preferred embodiments ethanol or methanol is used to achieve the advantageous double function as lignin solvent and salt anti-solvent. Other examples are ethylene glycol, diethylene glycol, glycerol or benzyl alcohol or lignin derived monomeric or oligomeric phenolics.

The anti-solvent function results in an improved salt removal since no additional step, such as a precipitation step, is needed before filtration. Another advantage of using e.g. ethanol or methanol is that it enables the use of a lower pH, such as pH < 4.5, without problems with lignin aggregates ("lumps").

As a product from the work-up and/or purification steps, a bio-oil composition can be obtained. The bio-oil composition comprises depolymerized lignin and further organic components from the biomass residue. The bio-oil composition includes a high content of organic components from the lignocellulosic biomass residue. The molecular weight of the bio-oil (after drying) may be in the range of about 200 g/mol to about 2500 g/mol, preferably about 250 g/mol to about 2200 g/mol, more preferably about 700 g/mol to about 2000 g/mol, most preferably about 800 g/mol to about 1800 g/mol. Determination of the average molecular weight may be performed as described in the Examples. According to an elemental analysis, the bio-oil (after drying) comprises about 35 to 45 wt% C, about 4.5 to about 5.5 wt% H, about 0.1 wt% or less N and about 25 to about 32 wt% O.

As a further product from the work-up and/or purification steps, an aqueous phase may be obtained. The aqueous phase includes liquefied carbohydrates from the lignocellulosic biomass residue such as organic acids, sugars, sugar derivatives and humins. These can be isolated in a separate process, e.g., using anti-solvent, ultrafiltration, nanofiltration or by non-selective water evaporation giving a carbohydrate rich oil or syrup.

According to particular embodiments of the present invention, the bio-oil composition is further subjected to distillation and/or hydrotreatment. By this means, biofuels may be produced in a high yield from lignocellulosic biomass residues. Hydrotreatment may, e.g., involve a treatment in the presence of a reducing gas such as H₂ and/or CO and a hydrotreatment catalyst at an elevated temperature, e.g., at a temperature between about 220°C to about 400°C, particularly between about 270°C and about 350°C. The product resulting from the hydrotreatment may be a hydrocarbon product containing only minor amounts of nitrogen, sulfur and/or oxygen.

Suitable bio-oil hydrotreatment procedures are described in co-owned patent applications WO 2017/078582 A1 and WO2020/161320 A1, the contents of which are herein incorporated by reference.

In a particular embodiment the process of the invention as described above is operated continuously.

The invention also relates to a lignin containing process stream obtainable by a process as described herein. Specifically, the lignin containing process stream according to the invention contains all turpentine and all methanol and all tall oil which is later part of the final bio-oil. The kraft mill black liquor used in the prior art does not contain any or at most traces of tall oil, turpentine and methanol. The reason for this is that turpentine and methanol are removed within the digester/cooker and the tall oil is skimmed off as tall oil soap. The resulting lean black liquor goes to the evaporators. The tall oil and turpentine are also called extractives and the total amount of extractives usually are 2-5% of dry wood, e.g. 2% for spruce and 5% for pine.

The invention also relates to a bio-oil composition obtainable by a process as described herein. In this respect, an oven dry bio-oil composition according to the invention has a melting point, whereas a commercial oven dry lignin powder does not. Compared to the prior art, the bio-oil composition according to the invention contains more cellulose/hemicellulose-based derivatives. Moreover, the bio-oil composition according to the invention contains all tall oil and all turpentine and all methanol available, whereas the lignin oil of the prior art does not contain tall oil, turpentine and methanol.

The melting point of the bio-oil composition according to the invention may lie in the range of about 120°C to about 180°C (at normal pressure), particularly in the range of about 130°C to about 170°C. In certain embodiments, the oil melting point may be about 130°C.

The bio-oil composition according to the invention will also contain salts, including, but not limited to sodium sulfate and/or sodium carbonate. The salt content may range, e.g., between about 15% (w/v) to about 20% (w/v). In exemplary embodiments, where ethanol is used as solvent, the bio-oil composition contains 15-20% salt as all salt is not removed with filtration. Lignin-oil according to the prior art contains only about 50 ppm salts.

The present invention is further defined by the following embodiments, which are part of the specification.
1. A method for producing a lignin-containing process stream, comprising the steps of:
   (a) providing a lignocellulosic biomass residue;
   (b) introducing the biomass into a reactor;
   (c) subjecting the biomass in the reactor to a treatment in the presence of an alkali source at elevated temperature, wherein the effective alkali charge is at least about 25 wt% on dry wood, wherein the temperature is at least about 150°C, and wherein the treatment time is at least about 1 h;
   (d) obtaining a lignin-containing process stream from the reactor; and
   (e) optionally removing char from the lignin-containing process stream.
2. The method of embodiment 1, wherein the lignocellulosic biomass residue is selected from sawdust, wood flour, wood chips, bark, branches, leaves, needles, or any mixture thereof.
3. The method of embodiment 1 or 2, wherein the lignocellulosic biomass residue is from softwood and/or hardwood.
4. The method of any one of embodiments 1-3, wherein the lignocellulosic biomass residue is introduced into the reactor without prior impregnation and in particular without acid impregnation.
5. The method of any one of embodiments 1-4, wherein the lignocellulosic biomass residue is introduced into the reactor without prior extraction using an organic solvent, e.g., an ethanol/water mixture.
6. The method of any one of embodiments 1-5, wherein a ratio of dry feed to liquid (w/w) from about 1:3 to about 1:10, particularly from about 1:4 to about 1:6, e.g., of about 1:5 is adjusted in the reactor.
7. The method of any one of embodiments 1-6, wherein the alkali source comprises Ba(OH)₂, NaOH and/or KOH.
8. The method of any one of embodiments 1-7, wherein the alkali source further comprises a sulfide salt, particularly sodium sulfide.
9. The method of any one of embodiments 1-8, wherein the alkali source is white liquor.
10. The method of any one of embodiments 1-9, wherein the effective alkali charge is at least about 30 wt% on dry wood, particularly from about 35 wt% on dry wood to about 60 wt% on dry wood.
11. The method of any one of embodiments 1-10, wherein the temperature in step (c) is about 150°C or higher, e.g., about 150°C to about 280°C.
12. The method of embodiment 11, wherein the treatment time is about 1 h to about 10 h.
13. The method of any one of embodiments 1-12, wherein step (c) is carried out under conditions of heat and treatment time resulting in a Kraft H factor of at least about 2000, at least about 4000, at least about 6000, at least about 7000, or at least about 8000.
14. The method of any one of embodiments 1-13, wherein step (c) is carried out under conditions of heat and treatment time resulting in a Kraft H factor of at most about 5 000 000, or at most about 3 000 000.
15.The method of any one of embodiments 1-14, wherein step (c) is carried out under conditions that the lignin-containing process stream obtained in step (d) or (e) comprises a low-grade solid pulp.
16. The method of embodiment 15, wherein the temperature in step (c) is between about 150°C and about 200°C, particularly between about 165°C to about 190°C, and more particularly between about 175°C to about 180°C.
17. The method of embodiment 15 or 16, wherein the treatment time is about 1 h to about 8 h.
18. The method of any one of embodiments 15-17, wherein the H factor is in the range of about 2000 to about 13000, particularly in the range of about 8000 to about 12000.
19. The method of any one of embodiments 15-18, wherein the yield of solid pulp is from about 20% to about 45% based on dry feed of lignocellulosic biomass residue.
20. The method of any one of embodiments 15-19, wherein the pulp has a Kappa number of about 50 or less, particularly of about 30 or less, more particularly of about 5 to about 20.
21. The method of any one of embodiments 15-20 further comprising separating the pulp from the lignin-containing process stream.
22. The method of embodiment 21 further comprising processing the pulp to sugar, biofuel such as ethanol, and/or biochemicals such as furan dicarboxylic acid (FDCA).
23. The method of any one of embodiments 1-14, wherein step (c) is carried out under conditions that the lignin-containing process stream obtained in step (d) or (e) does not comprise a substantial amount of solid pulp.
24. The method of embodiment 23, wherein the lignin-containing process stream obtained in step (d) or (e) contains about 5% (w/w) or less or about 1% (w/w) or less of solid pulp, particularly about 0.1% (w/w) or less of solid pulp.
25. The method of embodiment 23 or 24, wherein the temperature is about 200°C or higher, particularly from about 200°C to 280°C, and more particularly from about 210°C to about 240°C.
26. The method of any one of embodiments 23-25, wherein the treatment time is about 1 h to about 10 h.
27. The method of any one of embodiments 23-26, wherein the H factor is in the range of about 2000 and about 3 000 000, particularly in the range of about 2000 to about 1 000 000 or about 2000 to about 500 000, more particularly in the range of about 8000 to about 1 000 000, more particularly in the range of about 9000 to about 750 000, more particularly in the range of about 10000 to about 500 000.
28. The method of any one of embodiments 1-27, wherein the lignin-containing process stream obtained in step (d) or (e) is a black liquor, particularly a black liquor which comprises an increased amount of dissolved organic matter.
29. The method of any one of embodiments 1-28, wherein the lignin-containing process stream obtained in step (d) or (e) has a content of dissolved organic matter from about 60% to about 90%, particularly about 65% to about 90% based on the dry solids content within the process stream.
30. The method of any one of embodiments 1-29, wherein the lignin-containing process stream obtained in step (d) or (e) comprises about 30 weight-% to about 50 weight-%, preferably >33 weight-%, more preferably >40 weight-% lignin based on the dry solids content within the process stream.
31. The method of any one of embodiments 1-30, which is performed continuously.
32. The method of any one of embodiments 1-31, which is performed batch-wise.
33. The method of any one of embodiments 1-32 further comprising subjecting the lignin-containing process stream obtained in step (d) or (e) to a lignin-depolymerization step in a depolymerization reactor and obtaining a bio-oil containing process stream.
34. The method of embodiment 33 further comprising obtaining a bio-oil composition from the bio-oil containing process stream.
35. The method of embodiment 34 comprising one or more of the following steps:
   - acidifying the bio-oil containing process stream;
   - adding crude tall oil;
   - adding a solvent and anti-solvent such as ethanol, methanol, ethylene glycol, diethylene glycol, glycerol, benzyl alcohol or lignin derived monomeric or oligomeric phenolics, particularly ethanol or methanol;
   - removing an aqueous phase, solvent and/or salts from the bio-oil containing process stream.
36. The method of embodiment 35, wherein the step of acidifying the bio-oil containing process stream is carried out at a pH in the range of about 2 to about 5.
37. The method of any one of embodiments 34-36, further comprising subjecting the bio-oil composition to distillation and/or hydrotreatment.
38. A lignin-containing process stream obtainable by a process of any one of embodiments 1-32.
39. Use of the lignin-containing process stream of embodiment 38 for the manufacture of a bio-oil composition.
40. A bio-oil composition obtainable by a process of any one of embodiments 34-36.
41. Use of the bio-oil composition of embodiment 40 for the manufacture of a biofuel.

### Legends to the Figures

**Figure 1****:** Comparison of black liquor obtained according to the invention (A), namely according to Example 2.1 below, and black liquor from a conventional kraft pulp mill (B).
**Figure 2****:** Comparison of dried black liquor obtained according to the invention (A), namely according to Example 2.1 below, and black liquor from a conventional kraft pulp mill (B). Liquid samples to dry were extracted from bulk liquor and not from the surface.

### Examples

### Example 1: Small batch reactor experiments

### Example 1.1:

10 g milled softwood sawdust (including 5% moisture) and 100 g Kraft mill white liquor were added to a 300 ml reactor. The resulting slurry was heated for 5 h at 180°C during 250 rpm magnetic stirring. The heat treatment liquefied most sawdust and produced 1.72 g char (dry weight corresponding to 18% of the total dry sawdust) which was filtered off.

### Example 1.2:

10 g milled softwood sawdust (including 5% moisture) and 100 g Kraft mill white liquor were added to a 300 ml reactor. The slurry was heated for 5 h at 200°C during 250 rpm magnetic stirring. The heat treatment liquefied most sawdust and produced 0.32 g char (dry weight corresponding to 3.4% of the total dry sawdust) which was filtered off.

The pH of black liquor produced was 13.9. The black liquor was acidified to pH 4.5 to protonate the lignin. Then, the black liquor was extracted with the solvent ethyl acetate to separate any depolymerized lignin oil (bio-oil). This gave almost no product which indicates the need for a further depolymerization step with higher temperatures, e.g., 230-300°C.

### Example 1.3:

10 g milled softwood sawdust (including 5% moisture) and 100 g Kraft mill white liquor were added to a 300 ml reactor. This slurry was heated for 2 h at 230°C during 250 rpm magnetic stirring. The heat treatment liquefied most sawdust and produced 1.22 g char (dry weight corresponding to 12.8% of the total dry sawdust) which was filtered off.

Increasing the temperature from 200°C to 230°C gave more char despite the shorter reaction time.

### Example 1.4:

10 g milled softwood sawdust (including 5% moisture) and 100 g Kraft mill white liquor were added to a 300 ml reactor. The slurry was heated for 5 h at 155°C during 250 rpm magnetic stirring. The heat treatment provided a pulp and black liquor. The pulp was filtered off and the dry weight of the pulp was 7.35 g, which equals 77% of the total dry sawdust.

The black liquor was heated for 2 h at 230°C in a second step to depolymerize the lignin within the black liquor. Sulfuric acid (12.8 g) was used to acidify the 77.7 g heat treated black liquor to reach pH 4.5. The acid consumption was 165 kg/ton black liquor. Ethyl acetate (500 g) was added to extract the depolymerized lignin oil (bio-oil) by phase separation. The dry weight of bio-oil was 1.95 g. As the lignin content of softwood is 27% this gave a bio-oil yield of 77% based on the lignin content and a yield of 21% based on total dry biomass.

### Example 1.5:

62.5 g milled softwood sawdust, 250 g Kraft mill white liquor and 250 g water were added to a 2 L reactor. This was a liquid/solid ratio of 8.4 which gave a 10.6 wt% slurry. The slurry was heated for 5 h at 200°C during 600 rpm mechanical stirring. The heat treatment liquefied most sawdust and produced 7.8 g char (dry weight corresponding to 13.1% of the total dry sawdust) which was filtered off.

200 g of the resulting black liquor comprising liquefied sawdust was heat treated for 2 h at 230°C to depolymerize the lignin further. This liquor was acidified with sulfuric acid and the acid consumption to reach pH 4.5 was 57.9 kg acid/ton liquor. 500 ml ethyl acetate was added to extract the depolymerized lignin oil by phase separation and decanting. Filtering the water phase gave 0.9 g dry solids on filter paper. Final dry bio-oil weight was 5.7 g, which equals 24.8% yield of dry biomass.

### Example 1.6:

10 g (8.7 g dry ash-free bark) milled bark and 100 g Kraft mill white liquor were added to a 300 ml reactor. This slurry was heated for 5 h at 200°C during 250 rpm magnetic stirring. This heat treatment liquefied most (91%) bark and produced 9% char. The char contained 27% ash.

Char was filtrated off and the liquefied bark (pH 13.9) was acidified to pH 3 with 1:1 mass ratio of ethanol present. The precipitated sodium sulfate was filtered off. Salt recovery was 88% based on added sulfuric acid. The filtrate contained most organics from the liquefied bark as the precipitated salt only contained 1.2% organics. The filtrate was dried to obtain dry bio-oil. The weight of dry bio-oil was 8.0 g including 26% ash. The dry bio-oil yield based on dry ash-free bark was 68%.

### Example 1.7:

10 g (8.7 g dry ash-free bark) milled bark and 100 g KOH liquor (123 g/l concentration) were added to a 300 ml reactor. This slurry was heated for 5 h at 200°C during 250 rpm magnetic stirring. This heat treatment liquefied most (94%) bark and produced 6% char. The char contained 35% ash. Char was filtrated off and the liquefied bark (pH 14) was acidified to pH 3 with 1:1 mass ratio of ethanol present. The precipitated potassium sulfate was filtered off and the salt recovery was 85% based on added sulfuric acid. The filtrate contained most organics from the liquefied bark as the precipitated salt only contained 1.6% organics. The filtrate was dried to obtain dry bio-oil. The weight of dry bio-oil was 6 g including 9.4% ash. The dry bio-oil yield based on dry ash-free bark was 64%.

### Example 2: Pilot cooker experiments

These examples were performed in a pilot digestion reactor in which a continuous process can be simulated. The pilot cooking examples 2.1-2.5 are also summarized together with data from further examples in the table below. In the table below, reference 1 corresponds to example 2.1 and so on.

### Example 2.1:

3191 g wet (47% solids content) softwood sawdust was added to a cooking digester utilizing a fixed bed of sawdust and a circulating Kraft mill white liquor. 3.75 l white liquor was added to the system giving a liquid/solid ratio of 5/1. The alkali concentration was 33% on dry sawdust or 7.7 mol NaOH / kg dry sawdust. The sawdust was cooked for 6 h at 178°C giving a H factor of 9900. The pulp yield was 33% and the kappa number of the pulp was 8.1 giving an estimate of the lignin content of 1.2% within the pulp. The resulting black liquor had a residual alkali content of 10.3 g/l.

The black liquor was heat treated for 1 h at 230°C. Sulfuric acid was added to the lignin containing liquor to reach pH 5 followed by adding ethanol in 1:1 mass ratio. The produced slurry was filtered to remove sodium sulfate. The sodium sulfate recovery was 85% based on added acid and it contained 5% organics. The filtrate was dried to obtain 24.5 g dry oil including 27% ash. Molecular weight of the lignin containing bio-oil was analyzed to be 1480 Da using the method of dissolving the bio-oil in sodium hydroxide. Dry bio-oil started to melt at 130°C using the method of heating the bio-oil on a glass plate and detecting the melting point with an IR thermometer.

By this example, it can also be demonstrated that an increased content of dissolved organic matter is present in the black liquor obtained. The starting amount of dry wood is 1499.7 g (3191 g*0.47) and 33% pulp yield gives 494.9 g pulp. As indicated above, in this pulp 1.2% lignin are present, which gives 5.94 g lignin in the pulp. Lignin in the starting material is 28% (literature value) of dry wood, i.e., 0.28*1499.7 g dry wood which is 419.92 g lignin. So, by difference the lignin in black liquor is 419.92 - 5.94 = 413.98 g.

In a kraft mill, the lignin content in the pulp is 4.62% and the pulp yield is 50%. This gives 0.5*1499.7 g pulp which is 749.85 g pulp. 4.62% lignin in this pulp gives 34.64 g lignin within the pulp. Lignin in starting material is the same, 419.92 g so lignin in black liquor is by difference, 419.92-34.64 g = 385.28 g lignin. This is less than 413.98 g from harsh cooking according to the present invention. Accordingly, the harsh cooking gives 7.4% more lignin in the black liquor.

### Example 2.2:

3191 g wet (47% solids content) softwood sawdust was added to a cooking digester utilizing a fixed bed of sawdust and a circulating liquor. 2.58 l sodium hydroxide (261.2 g/l solution) was added to the system giving a liquid/solid ratio of 5/1. The alkali concentration was 45% on dry sawdust or 11 mol NaOH / kg dry sawdust. The sawdust was cooked for 8 h at 178°C giving a H factor of 13433. The pulp yield was 23% and the kappa number of the pulp was 5.6 giving an estimate of the lignin content of 0.9% within the pulp. The obtained black liquor had a residual alkali content of 25.5 g/l.

The black liquor was heat treated for 1 h at 230°C. Sulfuric acid was added to the lignin containing liquor to reach pH 5 followed by adding ethanol in 1:1 mass ratio. The produced slurry was filtered to remove sodium sulfate. The sodium sulfate recovery was 57% based on added acid and it contained 6% organics. The filtrate was dried to obtain 31.4 g dry oil including 30% ash. Dry bio-oil started to melt at 140°C using the method of heating the bio-oil on a glass plate and detecting the melting point with an IR thermometer.

### Example 2.3:

3191 g wet (47% solids content) softwood sawdust was added to a cooking digester utilizing a fixed bed of sawdust and a circulating liquor. 1.44 l sodium hydroxide (261.2 g/l solution) was added to the system giving a liquid/solid ratio of 5/1. The alkali concentration was 25% on dry sawdust or 6.2 mol NaOH / kg dry sawdust. The sawdust was cooked for 1.5 h at 178°C giving a H factor of 2494. The pulp yield was 50% and the kappa number of the pulp was 47.7 giving an estimate of the lignin content of 7.4% within the pulp. The obtained black liquor had a residual alkali content of 15.2 g/l.

### Example 2.4:

3191 g wet (47% solids content) softwood sawdust was added to a cooking digester utilizing a fixed bed of sawdust and a circulating liquor. 2 l potassium hydroxide (310 g/l solution) was added to the system giving a liquid/solid ratio of 5/1. The alkali concentration was 50.4% on dry sawdust or 9 mol KOH / kg dry sawdust. The sawdust was cooked for 6 h at 178 °C giving a H factor of 10835. The pulp yield was 34.8% and the kappa number of the pulp was 12.5 giving an estimate of the lignin content of 1.9% within the pulp. The obtained black liquor had a residual alkali content of 10.3 g/l.

The black liquor was heat treated for 1 h at 230 °C. Sulfuric acid was added to the lignin containing liquor to reach pH 5 followed by adding ethanol in 1:1 mass ratio. The produced slurry was filtered to remove potassium sulfate. The potassium sulfate recovery was 95% based on added acid and it contained 10% organics. The filtrate was dried to obtain 24.7 g dry oil including 26% ash. Molecular weight of the lignin containing bio-oil was analyzed to be 1740 Da using the method of dissolving the bio-oil in sodium hydroxide. Dry bio-oil started to melt at 170 °C using the method of heating the bio-oil on a glass plate and detecting the melting point with an IR thermometer.

### Example 2.5:

4054 g wet (37% solids content) softwood bark was added to a cooking digester utilizing a fixed bed of sawdust and a circulating liquor. 2 l potassium hydroxide (310 g/l solution) was added to the system giving a liquid/solid ratio of 5/1. The alkali concentration was 41.4% on dry bark or 7.4 mol KOH / kg dry bark. The sawdust was cooked for 6 h at 178 °C giving a H factor of 10264. The pulp yield was 32.7% and the kappa number of the pulp was not possible to determine hence not possible to estimate lignin content by kappa number. Lignin analysis was utilized giving a lignin content of 16% lignin within the pulp. The obtained black liquor had a residual alkali of 9.9 g/l.

The black liquor was heat treated for 2 h at 230 °C. Sulfuric acid was added to the lignin containing liquor to reach pH 5 followed by adding ethanol in 1:1 mass ratio. The produced slurry was filtered to remove potassium sulfate. The potassium sulfate recovery was 95% based on added acid and it contained 11% organics. The filtrate was dried to obtain 25.0 g dry oil including 23% ash. Molecular weight of the lignin containing bio-oil was analyzed to be 1730 Da using the method of dissolving the bio-oil in sodium hydroxide. Dry bio-oil started to melt at 125 °C using the method of heating the bio-oil on a glass plate and detecting the melting point with an IR thermometer.

### Summary of pilot cooker experiments

Table 1 summarize the pilot cooker trials and contain results from further pilot cooker trials. Reference no. 1 in the table below refers to pilot cooker trial example 2.1 and so on. Reference nos. 6-14 relate to examples, which are not described above in detail.

**Table 1:**

| **Ref.** | **Batch** | **Feed** | **Dry feed (kg)** | **Liquid volume (I)** | **Cooking time (min)** | **Cooking temperature (°C)** | **H-factor** | **Alkali source** | **Effective alkali charge (%)** | **Residual alkali (g/l)** | **Pulp yield (%)** | **Kappa number** | **Lignin in pulp (%)** |
|---|---|---|---|---|---|---|---|---|---|---|---|---|---|
| 1 | 4878 | Sawdust | 1.5 | 7.5 | 360 | 178 | 9900 | White liquor | 30% | 10.3 | 33 | 8.1 | 1.2 |
| 2 | 4879 | Sawdust | 1.5 | 7.5 | 480 | 178 | 13433 | NaOH | 45% | 25.5 | 23 | 5.6 | 0.9 |
| 3 | 4880 | Sawdust | 1,5 | 7.5 | 90 | 178 | 2494 | NaOH | 25% | 15.2 | 50 | 47.7 | 7.4 |
| 4 | 4881 | Sawdust | 1,5 | 7.5 | 360 | 178 | 10835 | KOH | 50% | 10.3 | 35 | 12.5 | 1.9 |
| 5 | 4882 | Bark | 1,5 | 7.5 | 360 | 178 | 10264 | KOH | 59% | 9.9 | 33 | - | 16 |
| 6 | 4883 | Sawdust | 1,5 | 7.5 | 360 | 178 | 11106 | KOH | 37% | 6.1 | 40 | 16.4 | 2.5 |
| 7 | 4884 | Sawdust | 1,5 | 7.5 | 330 | 178 | 10216 | KOH | 39% | 9.6 | 37 | 15.5 | 2.4 |
| 8 | 4885 | Sawdust | 1,5 | 7.5 | 383 | 178 | 11187 | KOH | 39% | 8.3 | 36 | 13.1 | 2.0 |
| 9 | 4886 | Sawdust | 1,5 | 7.5 | 420 | 178 | 12139 | KOH | 39% | 7.8 | 36 | 12.3 | 1.9 |
| 10 | 4887 | Sawdust | 1,5 | 7.5 | 353 | 178 | 10276 | KOH | 37% | 8.3 | 39 | 15.7 | 2.4 |
| 11 | 4889 | Sawdust | 1,5 | 7.5 | 420 | 176 | 11000 | White liquor | 39% | 17.7 | 27 | 5.9 | 0.9 |
| 12 | 4894 | Bark | 1,5 | 7.5 | 420 | 177 | 11000 | White liquor | 59% | 32.3 | 39 | - | - |
| 13 | 4896 | Sawdust | 1,5 | 7.5 | 390 | 177 | 11094 | KOH | 52% | 23.5 | 26 | 7.9 | 1.2 |
| 14 | 4897 | Sawdust | 1,5 | 7.5 | 390 | 178 | 11087 | NaOH | 39% | 23.5 | 27 | 8.2 | 1.3 |

The data presented in the above Table can be compared to a regular Kraft pulp which, directly after the digester commonly has a pulp yield in the range of 45-55% and a Kappa number of about 25-90. In the common Kraft pulping process, the conditions are gentler regarding temperature and alkali charge.

Table 2 summarizes and compares data for producing a lignin containing process stream and Table 3 for the work-up after a depolymerization step. The abbreviations are explained and connected to examples below.

**Table 2:**

| **Trial** | **Alkali / kg dry biomass (mol)** | **Alkali / dry biomass (wt%)** | **Pulp yield (wt%)** | **Temp. (°C)** | **Time (hr)** | **H factor** | **Kappa #** | **Lignin in pulp (wt%)** | **Residual alkali in black liquor (q/l)** | **Tall oil soap in black liquor (kg/ton dry solids)** |
|---|---|---|---|---|---|---|---|---|---|---|
| S/WL | 7.7 | 33.0 | 36 | 178 | 6 | 9900 | 8.1 | 1.25 | 10.3 | 1.0 |
| S/NaOH_s | 11 | 44.9 | 25 | 178 | 8 | 13433 | 5.7 | 0.9 | 26.0 | 1.3 |
| S/NaOH_w | 6,2 | 25.0 | 51 | 178 | 1.5 | 2494 | 47.5 | 7.3 | 15.0 | - |
| S/KOH_s | 9.0 | 50.4 | 35 | 178 | 6 | 10835 | 12.5 | 1.9 | 10.3 | 3.5 |
| B/KOH_w | 7.4 | 41.4 | 33 | 178 | 6 | 10264 | - | 16.0 | 9.9 | 20.7 |

**Table 3:**

| **Trial** | **Salt recovery (%)** | **Organics in salt (%)** | **Bio-oil Mw (Da)** | **Bio-oil m.p. (°C)** |
|---|---|---|---|---|
| S/WL | 85 | 5 | 1480 | 130 |
| S/NaOH_s | 57 | 6 | - | 140 |
| S/NaOH_w | - | - | - | - |
| S/KOH_s | 95 | 10 | 1740 | 170 |
| B/KOH_w | 95 | 11 | 1730 | 125 |

| | | | | |
|---|---|---|---|---|
| Abbreviations: S/WL - Sawdust/ White Liquor - Example 2.1 S/NaOH_s = Sawdust with strong NaOH - Example 2.2 S/NaOH_w = Sawdust with weak NaOH - Example 2.3 S/KOH_s = Sawdust with strong KOH - Example 2.4 B/KOH_w = Bark with weak KOH - Example 2.5 | | | | |

The lower pulp yield provided by the harsher cooking conditions results in an increased amount of organic matter within the black liquor and later within the bio-oil as essentially all organics (even water-soluble compounds and the extractives) end up within the bio-oil. This particularly applies when a solvent, e.g., ethanol, is added before or during acidification.

The use of sawdust/white liquor (Example 2.1) gave a pulp yield of 33%. This is an increase of about 15% organic matter within the black liquor compared to a conventional Kraft pulping process.

The use of sawdust/NaOH (Example 2.2) gave a pulp yield of 23%. This is an increase of about 25% organic matter within the black liquor compared to a conventional Kraft pulping process.

The use of sawdust/KOH (Example 2.3) gave a pulp yield of 35%. This is an increase of about 13% organic matter within the black liquor compared to a conventional Kraft pulping process.

The use of bark/KOH (Example 2.3) gave a pulp yield of 33%. This cannot be directly compared as there is no Kraft mill process for bark. It was found, however, that bark black liquor is high on sugars and extractives compared with black liquor from the other Examples.

The molecular weight of the produced bio-oils after a depolymerization step is significantly lower than conventional lignin powder from a Kraft mill having molecular weights in order of 4000-5000 Da. Using white liquor is more efficient to depolymerize the bio-oil giving a lower molecular weight compared with KOH media.

The produced bio-oils have a melting point in an open atmosphere, which is different to conventional lignin powder from a Kraft mill. A melted oil is easier to process further.

Table 4 shows elemental analysis results of dry oils.

**Table 4:**

| **Trial** | **C (%)** | **H (%)** | **N (%)** | **S (%)** | **O (%)** |
|---|---|---|---|---|---|
| S/WL | 39 | 4.8 | 0 | 2.0 | 27 |
| S/NaOH_s | - | - | - | - | - |
| S/NaOH_w | 38 | 5.0 | 0 | 0 | 27 |
| S/KOH_s | 38 | 4.8 | 0 | 0.8 | 30.6 |
| B/KOH_w | 43 | 5.3 | 0.1 | 0 | 28.3 |

The results support the presence of increased **amounts** of organic matter derived from cellulose and hemicellulose within the final bio-oil. The oxygen content (calculated by difference) is high compared to oil obtained from Kraft mill black liquor (25% oxygen) which indicates more oxygen-containing organic components within the bio-oil.

### Example 3: Comparison of black liquor samples

An optical comparison of a sample of black liquor obtained according to the invention (Fig. 1A; cf. Example 2.1 and Ref.1 in Table 1 above) and a sample of black liquor from a conventional kraft pulp mill (Fig. 1B) has been carried out. As can be seen, the black liquor obtained according to the invention has streams of substances on top of the black liquor whereas the kraft mill black liquor has no substances at the surface. The reason for this is, as indicated above, that the black liquor according to the invention still contains turpentine, methanol and tall oil, which is removed during manufacturing of the prior art black liquor.

When the black liquors are dried, the black liquor according to the invention (Fig. 2A; cf. Example 2.1 and Ref.1 in Table 1 above) shows a more gold-brown color which reflects the color of tall oil, turpentine and cellulose/hemicellulose-based derivatives, whereas the kraft mill black liquor (Fig. 2B) is black. Liquid samples to dry were extracted from bulk black liquor and not from the surface.

## Claims

1. A method for producing a lignin-containing process stream, comprising the steps of:
(a) providing a lignocellulosic biomass residue;
(b) introducing the biomass into a reactor;
(c) subjecting the biomass in the reactor to a treatment in the presence of an alkali source at elevated temperature, wherein the effective alkali charge is at least about 25 wt% on dry wood, wherein the temperature is at least about 150°C, and wherein the treatment time is at least about 1 h;
(d) obtaining a lignin-containing process stream from the reactor; and
(e) optionally removing char from the lignin-containing process stream.

2. The method of claim 1, wherein the lignocellulosic biomass residue is selected from sawdust, wood flour, wood chips, bark, branches, leaves, needles, or any mixture thereof; and/or
wherein the lignocellulosic biomass residue is introduced into the reactor without prior impregnation; and/or
wherein the lignocellulosic biomass residue is introduced into the reactor without prior extraction using an organic solvent, e.g., an ethanol/water mixture.

3. The method of claim 1 or 2, wherein a ratio of dry feed to liquid (w/w) from about 1:3 to about 1:10, particularly from about 1:4 to about 1:6, e.g., of about 1:5 is adjusted in the reactor.

4. The method of any one of claims 1-3, wherein the alkali source comprises Ba(OH)₂, NaOH and/or KOH and optionally a sulfide salt.

5. The method of any one of claims 1-4, wherein the effective alkali charge is at least about 30 wt% on dry wood, particularly from about 35 wt% on dry wood to about 60 wt% on dry wood.

6. The method of any one of claims 1-5, wherein the temperature in step (c) is about 150°C or higher, e.g., about 150°C to about 280°C, and/or the treatment time is about 1 h to about 10 h.

7. The method of any one of claims 1-6, wherein step (c) is carried out under conditions of heat and treatment time resulting in a Kraft H factor of at least 2000 and/or at most about 3 000 000.

8. The method of any one of claims 1-7, wherein step (c) is carried out under conditions that the lignin-containing process stream obtained in step (d) or (e) comprises a low-grade solid pulp, particularly as determined by a Kraft H factor in the range of about 2000 to about 13000, particularly about 8000 to about 12000.

9. The method of claim 8, wherein the yield of solid pulp is from about 20% to about 45% based on dry feed of lignocellulosic biomass residue, and wherein the pulp particularly has a Kappa number of about 50 or less, particularly of about 30 or less, more particularly of about 5 to about 20.

10. The method of claim 8 or 9 further comprising separating the pulp from the lignin-containing process stream and optionally processing the pulp to sugar, biofuel such as ethanol, and/or biochemicals such as furan dicarboxylic acid (FDCA).

11. The method of any one of claims 1-7, wherein step (c) is carried out under conditions that the lignin-containing process stream obtained in step (d) or (e) does not comprise a substantial amount of solid pulp, particularly as determined by a Kraft H factor in the range of about 2000 to about 3 000 000, particularly about 8000 to about 1 000 000, more particularly about 9000 to about 750 000, more particularly about 10000 to about 500 000.

12. The method of any one of claims 1-11, wherein the lignin-containing process stream obtained in step (d) or (e) is a black liquor.

13. The method of any one of claims 1-12 further comprising subjecting the lignin-containing process stream obtained in step (d) or (e) to a lignin-depolymerization step in a depolymerization reactor and obtaining a bio-oil containing process stream and obtaining a bio-oil composition from the bio-oil containing process stream.

14. The method of claim 13 further comprising subjecting the bio-oil composition to distillation and/or hydrotreatment.

15. A bio-oil composition obtainable by the method of claim 13.
